

July 27, 1937.

E. SEMMLER

2,088,389

METHOD OF PRODUCING BEARINGS

Filed March 7, 1935

Fig. 1



Fig. 2



Fig. 3



Fig. 5



Fig. 4



E. Semmler  
Inventor

By: Glascock Downing & Seebold  
A.H.S.

## UNITED STATES PATENT OFFICE

2,088,389

## METHOD OF PRODUCING BEARINGS

Erich Semmler, Berlin-Oberschoneweide,  
GermanyApplication March 7, 1935, Serial No. 9,885  
In Germany February 6, 1934

4 Claims. (Cl. 29—149.5)

This invention relates to an improved method for the production of bearings and has reference to bearings for high speed shafts, especially for aeroplane engines.

Recently such bearings have been constructed with a shell of steel lined with an alloy of copper and lead, the intention being that the steel shall provide the necessary strength and the alloy of copper and lead the characteristics required of a good bearing.

For this purpose alloys comprising from 80 to 60 parts of copper and from 20 to 40 parts of lead are employed, but, as these alloys show in the course of manufacture a strong tendency to liquation, i. e., for concentration of the lead to take place at certain parts, their serviceability is thereby greatly reduced, if not completely destroyed.

To prevent these local concentrations of lead the bearing must be chilled abruptly immediately after lining with the lead-copper alloy, but this chilling hardens the steel of which the bearing shells are made and thus makes machining and working much more difficult and gives the completed bearing, in certain circumstances, an undesirable brittleness which reduces its durability or makes it quite unsuitable for use with engines which have high demands put upon them.

To avoid the difficulties which arise due to the hardening of the steel, used for the bearing shells hitherto, during the chilling operation this invention provides for the use of non-hardenable iron for such bearing shells. It has been ascertained that non-hardenable iron suitable for this purpose must contain not more than 0.3% carbon, 0.3% silicon and 0.6% manganese. The silicon and the manganese may not be present in the composition and, when either or both of these substances are lacking, a somewhat higher carbon content may be present. However the important point is that under all circumstances the iron used for the bearing shells is not hardenable, so that in the necessary chilling for the prevention of lead liquation the iron experiences no noteworthy increase in hardness.

For the production of good bearings naturally it is of paramount importance that the bearing shell and the lining shall be joined together intimately, so that they form, as it were, one unitary piece and do not separate under the stresses of running. There is a difficulty, however, in the way of this intimate connection, since the melting point of the metal which is used for the shells differs greatly from that of the suitable bearing alloy. In order to overcome this diffi-

culty it has been proposed that the bearing shells should be given a thin coating of copper. This is not, however, in itself sufficient to produce the desired effect, care must also be taken to prevent the accession of air to the parts to be joined together from the time of the commencement of the necessary warming of the bearing shell up to the termination of the lining process.

This invention overcomes the above difficulty and achieves the desired result by first heating the bearing shell up to a temperature of about 1050° C. to 1085° C., which has been found to be suitable, in a bath of molten borax and leaving the bearing shell in such bath for a sufficient time. By this means not only is the shell brought up to the temperature stated above but also it receives simultaneously a coating which protects it reliably against oxydation. Before being put into the molten borax the bearing shell to be lined may be provided with a copper coating of from 1.5 to 2.5 mm. in thickness.

This invention then provides for the insertion of the prepared bearing shell into a mould with a base of graphite in which it is lined with the bearing alloy which has been melted meanwhile and for the prompt chilling of the mould and its contents when the molten metal has set. While effecting the chilling, care must be exercised to see that the water in the cooling tank into which the mould is thrown, and in which it is left until it is completely cold, does not reach too high a temperature to avoid which the cooling water is changed from time to time. Also it is desirable that the mould with its graphite base should likewise be warmed up before the molten bearing alloy is run in.

After cooling, the completed casting is in the form of a truncated cone, from which the bearing shell can be machined.

In the drawing:

Fig. 1 is a vertical section through a mould suitable for the purpose.

Fig. 2 is a side elevation of the mould shown in Fig. 1.

Fig. 3 is a detail view of the base of the mould.

Fig. 4 is a detail view of the clamp, and

Fig. 5 is a section through Fig. 3 taken on the line A—B.

As shown in the drawing, 1 is a cast iron mould with handles 2. The mould has a conical bore 50 and is provided at its base with an aperture 3; lugs 4, intended to cooperate with the ends of the clamp 5, are provided on the exterior of the mould, approximately at the height of the handles 2; 6 is the base of the mould which is made of

graphite and which has radially arranged grooves 1; and 8 is the overflow of the mould.

In the first place the two halves of a bearing shell are welded together with a gap between the edges of about 5 mm. as shown at 9 in Fig. 2, 5 and rendered completely clean with emery so as to remove completely the tempering colours originating from the welding. In the meantime an adequate sized crucible containing borax has been sufficiently heated to render the borax fluid. 10 The shell which preferably has been preheated to 50° C. is submerged in the molten borax in the crucible and left there for 2 to 3 minutes, after which the shell is taken out and placed exactly in the centre of the mould.

15 On the upper side of each shell a lug is formed, for example by milling and these lugs are arranged uppermost in the mould so as to be engaged by the upper parts of the retaining clamps 5, which embrace the lugs 4 by their lower ends 20 and thus prevent displacement of the shells during the operation of casting.

The introduction of the welded together pair of bearing shells into the mould must be effected as rapidly as possible, so that the temperature 25 of the bearing does not fall appreciably.

As soon as the pair of bearing shells have been secured by the two clamps 5, a metal alloy of the above mentioned kind, which has in the 30 meantime been melted and deoxydized in the well known manner, by means of phosphor copper, is run in.

Pouring is effected in the centre of the shells and such a quantity of molten metal should be used that about 3 kg. flows out by way of the 35 overflow 8. This metal which flows out can be caught in a mould made of dry sand and used for a subsequent cast.

Experience shows that bearings manufactured 40 in the manner described, in the first 50 hours of running, exhibit a considerable reduction of the lead bronze used as bearing metal, although it is not possible to discover metal particles in the oil.

Now it has been found that this disadvantage 45 can be overcome by the bored-out bushes being compressed by forcing a hard ball or a spherically ground mandrel through the bore. The compressing body is put through the bore of the bearing for the requisite number of times to attain the desired degree of compression.

As a result of this compressing step the improved bearing retains the amount of clearance which is given to it during manufacture, and the undesirable increase of clearance which occurs 50 with known bearings does not take place.

I claim:—

1. An improved method for the production of bearings having shells with a lining of a copper-lead alloy comprising forming the shells from iron not hardened by heat treatment, then heating said shells in a bath of molten borax up to a temperature of about 1050° C. to 1085° C., then inserting the heated shells into a mould, then casting therein a molten bearing alloy, and then chilling the mould and its contents by 10 plunging into cold water, and finishing the cold bearing to the desired dimensions after removal from the mould.

2. An improved method for the production of bearings having shells with a lining of a copper-lead alloy, comprising forming the shells from an alloy of iron containing up to 0.3% carbon, 0.3% silicon and 0.6% manganese; then heating said shells in a bath of molten borax up to a temperature of about 1050° C. to 1085° C., then inserting the heated shells into a mould, then casting therein a molten bearing alloy, and then chilling the mould and its contents by 20 plunging into cold water, and finishing the cold bearing to the desired dimensions after removal from the 25 mould.

3. An improved method for the production of bearings having shells with a lining of a copper-lead alloy, comprising forming the shells from iron not hardened by heat treatment, then heating 30 of said shells in a bath of molten borax up to a temperature of about 1050° C. to 1085° C., then inserting the heated shells into a mould, then casting therein a molten bearing alloy, and then chilling the mould and its contents by 35 plunging into cold water, and after removal of the bearing from the mould, machining the cold bearing and compressing the lining metal by the forced passage of a hardened mandrel through the bore.

4. An improved method for the production of bearings having shells with a lining of a copper-lead alloy, comprising forming the shells from an alloy of iron containing up to 0.3% carbon, 0.3% silicon and 0.6% manganese, then heating 45 said shells in a bath of molten borax up to a temperature of about 1050° C. to 1085° C., then inserting the heated shells into a mould, then casting therein a molten bearing alloy, and then chilling the mould and its contents by 50 plunging into cold water, and after removal of the bearing from the mould, machining the cold bearing and compressing the lining metal by the forced passage of a hardened mandrel through the bore.

ERICH SEMMLER.